

Oct. 30, 1945.

P. ALEXANDER

2,387,970

## THERMAL DEPOSITION OF METALS IN A VACUUM

Filed July 18, 1942

FIG. I.



6 F/G.2



FIG. 3.



FIG. 4.



FIG. 5.



*INVENTOR*

INVENTOR  
Paul Alexander

BY

BY  
Morrison, Kennedy & Campbell  
ATTORNEYS

ATTORNEYS

## UNITED STATES PATENT OFFICE

2,387,970

## THERMAL DEPOSITION OF METALS IN A VACUUM

Paul Alexander, Berkhamsted, England

Application July 18, 1942, Serial No. 451,468  
In Great Britain September 16, 1941

8 Claims. (Cl. 117—107)

This invention relates to the thermal deposition of metals in a vacuum.

In the process of thermal deposition in a vacuum, the metal to be deposited is heated to a temperature above its vaporisation point in a vacuum which may be from 0.00001 to 0.01 mm. Hg, depending on the process employed. The metal may be heated by a metallic heater or it may be heated in a non-metallic container. When a metallic heater is employed, the metal used for the heater must have a negligibly small vapour pressure at the temperature to which it is heated, so that no appreciable amount of this metal is vaporised to contaminate the vapour of the metal to be deposited.

Now the metals commonly required to be deposited are aluminium, copper, silver, gold and nickel, which require to be heated to 1000 degrees C. or over for their vaporisation. For metals with vaporisation temperatures of this order, the only metals available for use as heaters are the refractory metals, such as tungsten and molybdenum. Certain metals, and, in particular, aluminium, dissolve, or alloy with, the refractory metals at the temperatures employed, to a small extent, but enough to make them mechanically weak. Thus when, for instance, aluminium is brought into contact with the heater metal at a temperature adapted to the vaporisation of the aluminium, the heater breaks after a short time and has to be replaced. The life of a heater of the form commonly employed for vaporising aluminium is from ten to twenty minutes. The replacement of heaters entails re-evacuation of the chamber, which requires from half-an-hour to several hours, depending on the degree of vacuum employed. The process, therefore, is intermittent, and the interruptions entail much loss of working time.

However, in the specification of Patent No. 2,153,786 the applicant herein, described and claimed a process of thermal deposition in a vacuum of a metal to be evaporated in which this metal is fed as a wire or ribbon, end on, to a heater at such a rate that the metal is evaporated substantially as soon as it comes into contact with the heater and thereby the metal cannot lie on the heater in a molten state, thus, alloying is avoided and a continuous process thereby obtained, whilst loss of time in breaking and re-establishing the vacuum to effect repairs is entirely eliminated.

The main object of the present invention is to provide an improved continuous process of thermal evaporation of metals in which the vapour

density of the metal evaporated is kept low by evaporating it at all points of the surface of a liquid bath. Thereby the rate of evaporation may be made as large as desired, while still maintaining low vapour density, by increasing the surface area of the liquid bath.

A further object of the invention is to avoid the short life of solid heaters and the consequent expense of their replacement, and the loss of time in breaking and re-establishing the vacuum, due to the metal to be evaporated alloying with and destroying the heater, by the use of a liquid heater with which the metal is alloyed or mixed.

Accordingly the metal to be deposited may be fed to the liquid heater as a wire or ribbon, as in the case of aluminium, or may be fed to the mixture by dropping pellets or crystals of the metal into the liquid, as in the case of chromium, which metal cannot be drawn into wire form.

According to the present invention a process of depositing on a support a bright film of a metal selected from the group consisting of gold, nickel, cobalt, iron, copper, aluminium, chromium, and silver, which is deposited by thermal evaporation in a vacuum consists in continuously maintaining liquid a mixture of a metal, selected from the group consisting of platinum and palladium and a small percentage of the said metal to be evaporated, exposing said support to the vapour from said mixture, and maintaining the percentage of said metal to be evaporated approximately constant in said mixture by feeding the metal to be evaporated into the said mixture at a rate equal to the rate of evaporation of said metal to be evaporated.

Apparatus for carrying out the process according to the invention comprises in a vacuum chamber, a heater consisting of a bath of liquid platinum or palladium, a vessel adapted to contain the liquid bath and means for maintaining the platinum or palladium liquid, and means for feeding into the liquid bath the metal to be evaporated at a rate adjustable to maintain an approximately constant and small percentage of the metal to be evaporated in the liquid bath.

In a preferred form of apparatus according to the invention the vessel increases in cross section at its ends and the mixture is heated by electrodes of refractory metal, preferably tungsten, entering of the vessel, the cross section of the vessel where the container metal makes contact with the electrodes being sufficient to pass the heating current without melting, while the metals in the central portion of the bath are liquid.

The bath may be contained in a non-metallic vessel and may be heated either by high frequency induced current or by an electrically heated coil of refractory metal protected from contact with the molten metal in the bath and shielded from the vapour of the metal evaporated.

In order that the invention may be more clearly understood, preferred embodiments thereof will now be described with reference to the accompanying drawing, in which:

Figure 1 is a vertical section showing a vacuum chamber with thermal deposition apparatus;

Figure 2 is a vertical section to an enlarged scale of the non-metallic heating vessel shown in Figure 1;

Figure 3 is a plan of a modified form of the heating vessel of which

Figure 4 is a vertical section; and

Figure 5 is a sectional elevation of a pellet or powder dropping device.

In the drawing like references designate the same or similar parts.

Referring first to Figures 1 and 2 of the drawing, the vacuum chamber 1 contains the support 2 on which the metal is to be deposited, a liquid mixture 3 of platinum or palladium contained in a refractory vessel 4, for example of alumina, and a clockwork 5 adapted to feed at an adjustable rate a wire 6 of the metal to be deposited from a spool 7 into the bath 3. A screen 8 shields the neighbourhood of the point of contact between the wire 6 and the liquid 3, so as to protect the support from the denser vapour issuing from this point. Figure 2 shows, to an enlarged scale, the bath 3 of platinum or palladium contained in a vessel 4 of refractory material, such as alumina. Lugs 9 serve to support the vessel 4 on the brackets 10 (Figure 1). The bath is heated by a zig-zag coil 11 of refractory metal, such as tungsten, embedded in the refractory material 12 of the vessel 4 so that the coil is protected from contact with the molten metal and shielded from the vapour of the metal evaporated.

Figures 3 and 4 show an alternative form of heating vessel, in which the cross-section of the bath at the ends 13 is considerably larger than in the central channel and electrodes 14 of refractory metal enter the bath at the ends 13 so that the metal of the bath is partly liquid and partly solid.

Heating current is supplied through the electrodes 14 to heat the bath and the cross section of the bath at the ends 13 is sufficient to pass the heating current without melting the metal at the ends whilst the platinum or palladium in the relatively narrow central channel is liquid. As the metal at the ends is solid the electrodes 14 are at a temperature below that at which the vapour of the metal being deposited can alloy with them.

By forming the electrodes and if desired, also the ends of the bath with relatively large heat radiating surfaces, the temperature in the region of the electrodes, for a given current density, may be lowered, whereby minimum cross section of the ends of the bath may be attained, while still maintaining the metal in the ends of the bath in the solid state.

Figure 5 shows a device for dropping pellets or powder of the metal into the bath through the screen 8. The wheel 15, driven slowly by a clockwork similar to 5, is notched, and takes pel-

lets or powder from the hopper 16 and, as it turns, drops the pellets or powder into the bath at the predetermined rate of feed.

A small proportion of the metal to be evaporated is mixed with platinum, a convenient proportion being from three per cent to twenty per cent. The mixture is heated in the vessel 4 and maintained in a liquid condition, with liquid surface exposed to the support 2, for example made of glass or paper on which the metal is to be deposited.

Assuming, for example, that aluminium is being evaporated, and that a platinum-aluminium mixture containing about 7% aluminium is heated to about 1700 degrees C., the vapour pressure of the aluminium is then about 10 mm., and that of the platinum is about 0.0001 mm. of Hg. There is, therefore, no appreciable evaporation of the platinum, while the aluminium evaporates readily in a vacuum of 0.01 mm. of Hg. Since the proportion of aluminium to platinum is small, the vapour density of the aluminium at the surface of the liquid is low. The process is made continuous by feeding aluminium into the liquid mixture at a rate approximately equal to the rate at which the aluminium is evaporated, so that the mixture is maintained at approximately constant composition. The rate of feed is such as to ensure the aluminium liquifying and diffusing in the platinum without appreciable vapourisation.

The liquid mixture in the bath is kept substantially homogeneous by diffusion and by the convection currents in the liquid, apart from the region of somewhat higher concentration in the neighbourhood of the feeding point. The screen 8 serves also to prevent the vapour from this region from reaching the support 2.

By increasing the proportion in the liquid mixture of the metal to be evaporated, the rate of deposit is increased, but, at the same time, the vapour density is increased. It is, therefore, of advantage to increase the proportion, and so secure rapid working, while keeping the proportion below that which gives a dull deposit at the vacuum employed.

This adjustment, to obtain optimum working conditions in any given installation, can be made by adjusting the rate of feed of metal into the liquid mixture.

The word "mixture" has been employed to denote the combination of the metal to be deposited with the platinum. Since the mixture is operative only when liquid, it is immaterial whether one metal is alloyed with the other, or dissolved in it or merely mixed with it, and the word "mixture" is used to denote any one of the forms in which the metals can be combined when in liquid form.

The invention has the further advantage that the vapour density of the metal vapour can be kept as low as desired by adjusting the proportion of the metal to be evaporated in the bath. It is known that a film of good quality, having a bright surface, can be deposited only in a high degree of vacuum, of 0.001 to 0.0001 mm. Hg if the vapour density of the metal is high, and in the absence of special heating means for the vapour, but that, if the vapour density is kept low, a vacuum of only 0.01 to 0.001 mm. Hg is sufficient to obtain a bright film.

The following metals, among others, may be evaporated by the process the subject of the invention: gold, nickel, cobalt, iron, copper, aluminium, chromium, silver. In the case of chro-

mium, which cannot be drawn into wire, the feeding is effected by dropping pellets or crystals of the metal into the liquid.

Either platinum or palladium may be used as the metal with which the metal to be evaporated is mixed.

From the foregoing it will be observed that the invention comprises the operation of a continuous process for the thermal deposition of a metal from a liquid mixture comprising platinum or palladium, within which has been incorporated a small percentage of the metal to be evaporated, and the invention also covers the coated support produced in carrying out the process herein described.

I claim:

1. In a process of depositing on a support a bright film of a metal, selected from the group consisting of gold, nickel, cobalt, iron, copper, aluminium, chromium and silver, which is deposited by thermal evaporation in a vacuum, the steps of continuously maintaining liquid a mixture of a metal, selected from the group consisting of platinum and palladium, and a small percentage of the said metal to be evaporated, exposing said support to the vapour from said mixture, and maintaining the percentage of said metal to be evaporated approximately constant in said mixture by feeding the metal to be evaporated into the said mixture at a rate equal to the rate of evaporation of said metal to be evaporated.

2. A process according to claim 1 including the steps of proportioning the said metal to be evaporated to the metal selected from the group consisting of platinum and palladium in such a manner as to obtain a low vapour density of the said mixture, and evaporating the said mixture in a vacuum of 0.01 to 0.001 mm. Hg.

3. A process according to claim 1, wherein said mixture contains a proportion of from three to twenty per cent of said metal to be evaporated.

4. A process according to claim 1, wherein the said metal to be evaporated is aluminium, the said mixture containing about 7% thereof.

5. Apparatus for the thermal evaporation in a vacuum of metals of high vaporisation point, comprising a vacuum chamber, a heater in the chamber consisting of a bath of a liquid of a metal selected from the group consisting of platinum and palladium, a vessel adapted to contain the liquid bath and means for maintaining the bath liquid, and means for feeding into the liquid bath the metal to be evaporated at a rate adjustable

to maintain an approximately constant and small percentage of the metal to be evaporated in the liquid bath.

6. Apparatus for the thermal evaporation in a vacuum of metals of high vaporisation point, comprising a vacuum chamber, a heater in the chamber consisting of a bath of a liquid of a metal selected from the group consisting of platinum and palladium, a vessel adapted to contain the liquid bath, the vessel being of increased cross section at its ends, and heating electrodes of refractory metal entering the said ends of said vessel, the cross section of the vessel at the ends thereof being sufficient to enable a heating current supplied to the electrodes to pass through the metal in the said ends without melting it, whilst the metal intermediate the ends of the vessel is melted to form the liquid bath, and means for feeding into the bath the metal to be evaporated, at a rate adjustable to maintain an approximately constant and small percentage of the metal to be evaporated in the liquid bath.

7. Apparatus for the thermal evaporation in a vacuum of metals of high vaporisation point, comprising a vacuum chamber, a vessel of non-metallic material, a quantity of a metal selected from the group consisting of platinum and palladium in said vessel, means for continuously maintaining at least a portion of said quantity of metal liquid, whereby a bath of the liquid is contained in said vessel and constitutes a heater for the metal to be evaporated, means for feeding to the surface of the bath a length of wire of the metal to be evaporated and means for regulating the rate of feed of the wire to maintain an approximately constant and small percentage of the metal to be evaporated in the liquid bath.

8. Apparatus for the thermal evaporation in a vacuum of metals of high vaporisation point, comprising a vacuum chamber, a vessel of non-metallic material, a quantity of a metal selected from the group consisting of platinum and palladium in said vessel, means for continuously maintaining at least a portion of said quantity of metal liquid, whereby a bath of the liquid is contained in said vessel and constitutes a heater for the metal to be evaporated, said means including an electrically heated coil of refractory material embedded within the material of the vessel, and means for feeding into the liquid the metal to be evaporated at a rate adjustable to maintain an approximately constant and small percentage of the metal to be evaporated in the liquid bath.

PAUL ALEXANDER.

CERTIFICATE OF CORRECTION.

Patent No. 2,387,970.

October 30, 1945.

PAUL ALEXANDER.

It is hereby certified that error appears in the printed specification of the above numbered patent requiring correction as follows: Page 2, second column, line 66, for "0.001" read --0.0001--; and that the said Letters Patent should be read with this correction therein that the same may conform to the record of the case in the Patent Office.

Signed and sealed this 26th day of February, A. D. 1946.

Leslie Frazer *x*

(Seal)

First Assistant Commissioner of Patents.